

Feb. 28, 1933.

C. H. KERK

1,899,419

TANTALUM SPINNERET AND METHOD OF MAKING SAME

Filed Nov. 26, 1929

Fig. 1.



Fig. 2.



Fig. 3.

Fig. 4.



Fig. 5.

Fig. 6.



INVENTOR.

Charles H. Kerk

BY

Symmetcoedt & Dechner

ATTORNEYS

## UNITED STATES PATENT OFFICE

CHARLES H. KERK, OF ST. DAVIDS, PENNSYLVANIA

## TANTALUM SPINNERET AND METHOD OF MAKING SAME

Application filed November 28, 1929. Serial No. 410,006.

This invention relates to spinnerets such as are employed in the spinning of artificial silk thread.

The nature, objects and advantages of my invention will be understood from the following.

The spinneret most commonly employed in the artificial silk industry is of the thimble type, the crown of the thimble being flat and provided with the apertures or holes through which the cellulose or other solution is spun into the precipitating bath. The spinneret holes may be very fine, as fine, for example, as .002 of an inch in diameter, and the holes must be accurate to much less than .0001 of an inch. The number of holes in the crown varies with the number of filaments of the thread which is being spun. The solution is forced through the spinneret holes by means of an extrusion pump.

The spinnerets, therefore, are subjected to chemicals, to pressure, and to wear incident to the extrusion of the solution, in consequence of which the life of the spinneret is relatively short. Increase in size of the holes or distortion of the holes is very objectionable as it results in changes in the denier of the filaments.

Heretofore it has largely been the practice to make the spinnerets out of the precious metals or alloys thereof, such as gold and platinum and palladium. Insofar as spinnerets made from these metals or alloys are unaffected by the chemicals employed, they are satisfactory. However, they are relatively soft, wear rapidly, become distorted easily, and are susceptible to damage when being cleaned. They are also quite expensive.

It is the primary object of my invention to provide a spinneret which is free from the aforesaid objectionable characteristics, is not affected by the chemicals employed, has long life, and is inexpensive.

To this end I propose to make the spinnerets from the metal tantalum. Tantalum, as a practical matter, cannot be shaped in spinnerets by the dies because it does not flow and adheres to the dies and also causes the dies to wear so rapidly that only a few spinnerets can be made to size before the dies are

ruined. In order to make it commercially feasible to employ the metal tantalum for spinnerets, I first treat the metal—usually in sheet form for this purpose—so that it will readily flow in the dies without sticking and without shortening the life of the dies. The preferred treatment is to provide a film on the surface of the metal, this being done by immersing the metal in a mild iron sulphate solution through which an electric current is passed. Thereby an oxide forms on the surface in an immeasurably fine film. The presence of this film on the surface secures the results above set forth.

To illustrate an example of the various stages or steps in the production of the spinnerets, a sheet of drawings is appended, and on this sheet—

Figure 1 illustrates in section a suitable sheet of tantalum from which the spinnerets may be stamped; and

Figures 2 to 6 inclusive illustrate a spinneret, in section, at different stages of its manufacture.

Referring first to Figure 1, a strip or sheet of tantalum is indicated by the reference numeral 7. This figure also shows the oxide film at 8, formed at each side of the sheet 7 in accordance with the treatment above set forth, it being noted that the plate and the film are greatly exaggerated as to thickness for purposes of illustration.

The first operation in the actual production of the article includes preferably simultaneous stamping and forming of generally thimble shaped members having a substantially cylindrical wall 9 and a base 10 in which the spinneret holes will ultimately be drilled.

In the second die operation (see Figure 3) the shape of the thimble is somewhat altered by extending the cylindrical wall, as shown at 9a, and reducing the diameter thereof as well as of the head, as shown at 10a.

As seen in Figure 4, the next operation provides an outturned flange 11 at the open end of the cylinder 9a. The flange is then preferably trimmed to a uniform circular shape.

In accordance with Figure 5, the succeed-

ing die operation provides an upturned lip 12 or the like at the outer edge of the flange 11.

Finally, and as viewed in Figure 6, the spinneret is completely shaped by bending the upturned lip 12 downwardly adjacent to the remaining portion of the flange 11, for example, as shown at 12a.

In considering the foregoing figures, it should be noted that the oxide film is illustrated only in Figure 1, it being pointed out, however, that in accordance with this invention, the film serves to prevent sticking of the tantalum in the stamping dies and thus makes it possible to produce spinners from tantalum by such die stamping operations. After completion of the article, in accordance with the foregoing, the spinneret holes may be drilled in the head of the thimble.

I further discovered that a tantalum spinneret, after the holes have been formed therein, may be hardened without distortion or change in dimension of the spinneret or spinneret holes. Such a spinneret will withstand pressure, will wear much longer, will withstand cleaning without damage if ordinary care is exercised, is unaffected by the chemicals employed and is very much cheaper than the precious metal alloys heretofore employed. A more perfect product is ensured over a relatively long period of use.

To harden the spinners I subject them to heat, say from 500 to 1000 degrees Fahrenheit, preferably in the neighborhood of 850 degrees Fahrenheit. As a result of this treatment an oxide surface is developed which gives the desired hardness without injury to or imperfection in the perforations. The depth of the oxide is controlled by the length of time of heating. While the metal oxidizes under conditions just pointed out, it does not oxidize at low temperatures, and hence there is no danger that further oxide will be formed under the normal conditions of use.

The metal columbium is similar to tantalum and when subjected to the treatments above given, it may also be commercially produced in the form of spinners and the spinners hardened. The scope of this invention is, therefore, to be understood as including metals or alloys of metal which are similar in nature and behaviour to tantalum. The spinners also may be made in the form of capillaries, instead of the thimble type, and it is to be understood that the term "spinneret" is used in a broad sense.

I claim:

1. The herein described process of making spinners which consists in immersing a sheet composed of tantalum in an iron sulphate solution, in passing a current therethrough to form an oxide on the surface of the sheet, in stamping a spinneret from the

sheet and in heating the spinneret to oxidize the surface thereof.

2. The herein described process of manufacturing a spinneret from tantalum sheeting which includes the steps of immersing the sheeting in an electrolytic bath, whereby to produce an oxide coating on the surface of the sheeting, and die stamping the spinneret from the oxide coated sheeting. 70

3. The herein described process of manufacturing a spinneret from tantalum sheeting which includes the steps of immersing the sheeting in an electrolytic bath, whereby to produce an oxide coating on the surface of the sheeting, die stamping the spinneret from the oxide coated sheeting, and thereafter hardening the surface of the spinneret by heat treatment at a temperature preferably above 500° Fahrenheit. 75

4. The method of making an article from tantalum sheeting which includes immersing the sheeting in an electrolytic bath, effecting a flow of current between the bath and the sheeting to form an oxide film on the surface of the sheeting, and thereafter die stamping the article from the sheeting, whereby the normal tendency of the tantalum to stick in the stamping dies is substantially eliminated by virtue of the electrolytic treatment. 85

5. As a new article of manufacture, a spinneret composed of tantalum and having a multiplicity of small apertures or capillary openings therethrough, the surfaces of said capillary openings being hardened. 90

6. The method of manufacturing a spinneret from tantalum sheeting which includes forming a spinneret from the sheeting, drilling a multiplicity of apertures or capillary openings therethrough and thereafter hardening the surfaces of said capillary openings. 100

In testimony whereof I have hereunto signed my name.

CHAS. H. KERK.

110